

April 25, 1933.

A. L. J. QUENEAU

1,905,604

PROCESS OF ROASTING ORES

Filed June 25, 1931



INVENTOR

AUGUSTIN LEON JEAN QUENEAU.

BY

*Meissner & Rauher*

ATTORNEYS.

## UNITED STATES PATENT OFFICE

AUGUSTIN LEON JEAN QUENEAU, OF NEW YORK, N. Y.

## PROCESS OF ROASTING ORES

Application filed June 25, 1931. Serial No. 546,892.

This invention relates to metallurgy and more particularly to methods of treating ores and metal bearing materials to facilitate the recovery of the metal bearing constituents 5 therefrom.

Heretofore in the art it has been customary to subject ores and materials containing metal sulfides to an oxidizing roast to convert the sulfur and the metal contents thereof to oxide compounds. The sulfur oxides are gaseous and are carried off and recovered as sulfuric acid. The oxidized metal values are thereafter recovered from the roasted residues in any convenient manner.

15 In the oxidizing of zinc sulphide ore, it is customary to pass the ore through a roaster in order to liberate the sulfur and to bring about a transformation of the zinc sulphide to zinc oxide so that metallic zinc can be recovered therefrom by known methods of pyro-metallurgy.

20 In the oxidizing of zinc sulphide ore, it has been found that an excessive heat is developed at certain places within the roasting furnaces 25 which causes a detrimental fusing of the ore and brings about an agglomeration of the charge. This solidification or agglomeration interferes very materially with the operation of the furnace and requires frequent shutdowns for the purpose of breaking up the charge. Air cooling at such zones has been resorted to. This is objectionable as it increases the volume of outgoing gases and also increases the dust carrying capacity thereof.

30 It is one of the objects of the present invention to eliminate this detrimental fusing of the zinc sulfide ores during the oxidizing of the same.

35 Another object of the present invention is to improve the method of oxidizing zinc sulfide ores.

Another object of the present invention is to provide an improved type of ore roasting apparatus.

40 These and other objects and advantages will become apparent as the invention is more fully disclosed.

45 In accordance with the objects of the present invention I have found that this detrimental heating of the ore usually occurs with-

in the furnace between the fifth and seventh hearths (counting from the top) in a standard type of 16 hearth roasting furnace customarily used.

I have also found that this detrimental 55 heating may be overcome by introducing within the furnace and upon the hearth or hearths wherein this detrimental fusing occurs, a proportion of inert material, preferably of relatively high heat absorbing 60 value, thereby offsetting the tendency of the ore to liberate the excessive heat energy at this point.

The effluent furnace gases carry a relatively 65 large quantity of dust particles which are comprised of a relatively high proportion of zinc sulfate. To convert zinc sulfate into zinc oxide and sulfur oxide products a relatively large quantity of heat must be applied thereto. I propose therefore to recover the 70 dust product of the effluent gases of the furnace and to return the same to the furnace at the zone where excessive heating usually takes place thereby utilizing the endothermic 75 reaction of the thermal decomposition of the zinc sulphate content of the dust product to bring about a cooling of the ore under treatment at the critical zone. Before further disclosing the nature and scope of the present 80 invention, reference should be made to the following drawing wherein:

The figure is a vertical longitudinal section through a roasting furnace suitable for carrying out the method of the invention, the view also diagrammatically showing certain related apparatus for the collecting and reintroducing of the dust product into the 85 hot zone of the furnace.

Referring in detail to the drawing, 10 represents a roasting furnace of known construction which is usually provided with a plurality of superimposed shelf-like hearths 12 having central openings 14. Stirring arms 16 carried by a centrally disposed rotatable shaft 18 serve to feed the pulverized ore along the hearths. Fuel such as natural gas, city gas, oil or the like may be introduced within the furnace through a suitable burner 22.

The sulphide ore (ZnS) to be treated is 100

fed in through a suitable hopper 24 to the uppermost hearth. Then due to the rotation of the rabble arms 16 the charge is progressively fed from one shelf to another through 5 the opening 14.

The roasting furnace illustrated has 16 hearths. In practice, it has been found that the excessive heating takes place in the zone between the fifth and seventh hearth.

- 10 The heated and oxidizing gases arising in the furnace from burner 22 carry off a dust product containing a substantial proportion of zinc sulphate ( $ZnSO_4$ ). These gases and the entrained dust are taken off at the top of 15 the roasting furnace through a pipe 26 and led to a suitable dust separator 28. The dust is trapped in the separator and flows through a pipe 30 to a bin 31 and thence to a screw conveyor 32 which introduces the dust 20 containing the zinc sulphate onto the hearth located at the predetermined critical zone. A pipe 34 connected to the dust collector carries off the sulphur dioxide to a suitable apparatus (not shown) for the recovery of sulphuric acid.

The zinc sulfate content of the dust thus introduced is thermally decomposed by the heat energy of the furnace to form zinc oxide and sulfur oxides compounds. This 30 reaction is endothermic in nature and requires a relatively high temperature approximating 770° C. In addition the dust particles because they are relatively cold have a distinct cooling effect on the temperature of the 35 charge independent to the endothermic thermal decomposition reaction.

From the foregoing it will be readily apparent that according to my novel method the cooling of the charge of ore under treatment is brought about solely by introduction of the dust product recovered during normal treatment and without the introduction of any cooling air. Thus the cooling effect is secured without increasing the volume of 45 outgoing gases and consequently without multiplying the dust carrying capacity of such gases. The advantages which accrue as a result of the improved method will be readily appreciated by those skilled in the 50 art.

While I have described with great particularity certain specific steps in the preferred method it is not to be construed that I am limited thereto and the detailed description is to be interpreted in an illustrative rather than a limiting sense since various modifications may be made by those skilled in the art without departure from the scope of the invention as defined in the 55 appended claims.

What is claimed:

1. In the roasting of ores, the method of controlling the temperature of the roast which comprises adding at an intermediate point in the roasting process where the tem-

perature is excessive increments of thermally decomposable material of relatively high heat absorbing capacity.

2. In the roasting of ores, the method of controlling the temperature of the roast which 70 comprises adding at an intermediate point in the roasting process where the temperature is excessive during the roasting operation increments of thermally decomposable material of relatively high heat absorbing capacity. 75

3. In the roasting of zinc sulfide ores, the method of controlling the temperature of the roasting operation which comprises adding at an intermediate point in the roasting process 80 where the temperature is excessive increments of thermally decomposable material of relatively high heat absorbing capacity. 85

4. In the roasting of zinc sulfide ores, the method of controlling the temperature of the roasting operation which comprises adding at an intermediate point in the roasting process where the temperature is excessive increments of zinc sulfate. 90

5. In the roasting of zinc sulfide ores, the method of controlling the temperature of the roasting operation which comprises adding at an intermediate point in the roasting process where the temperature is excessive increments of material comprised in part of zinc 95 sulfate. 100

6. In the roasting of zinc sulfide ores the method of controlling the temperature of the roasting operation which comprises adding to the ore at a predetermined point in the furnace where the temperature during the roasting becomes excessive, a proportion of a material comprised at least in part of thermally decomposable material of relatively high heat absorbing capacity. 105

7. In the roasting of zinc sulfide ores the method of controlling the temperature of the roasting operation which comprises adding to the ore at a predetermined point in the furnace where the temperature during the roasting becomes excessive, a proportion of a material comprised at least in part of zinc sulfate. 110

8. In the roasting of zinc sulphide ore the method which includes the step of utilizing zinc sulphate ( $ZnSO_4$ ) to exert a cooling action on the ore at a predetermined point in the roasting furnace where the roasting temperatures become excessive. 115

9. A method of roasting zinc sulphide ore which comprises feeding the ore in a finely divided state through an atmosphere of hot oxidizing gases, collecting the resulting dust product containing zinc sulphate ( $ZnSO_4$ ) and returning said dust product to the ore under treatment at a predetermined zone where the roasting temperatures become excessive so as to utilize its endothermic reaction to effect a cooling of the ore at that zone. 125

10. In the roasting of zinc sulphide ore the 130

method which comprises feeding the finely divided ore successively over a plurality of hearths of a roasting furnace, subjecting the ore to the heat of reaction of an oxidizing gas

5 in the roasting furnace, carrying off the resulting gases and a fine dust product comprised at least in part of zinc sulphate, zinc oxide and gangue, collecting such dust product and reintroducing it at a predetermined zone of

10 the furnace where the roasting temperature becomes excessive to effect a cooling of the ore under treatment in said zone.

11. In the roasting of zinc sulphide ore, the method which comprises feeding finely divided ore gradually over the hearths of a roasting furnace, subjecting the ore to an atmosphere of oxidizing gases in said furnace, collecting a dust product carried off with the outgoing gases which product includes a substantial percentage of zinc sulphate, and mixing such dust product with the ore under treatment at a predetermined zone within the furnace where the roasting temperature become excessive so as to utilize the endothermic

20 reaction of the zinc sulphate content in the dust product to effect a reduction of temperature of the ore under treatment in said zone.

25

In witness whereof, I have hereunto signed my name.

30 AUGUSTIN LEON JEAN QUENEAU.

35

40

45

50

55

60